

March 30, 1937.

P. M. HALL

2,075,281

SMOKER'S PIPE

Filed Nov. 18, 1933



Irvinator  
Preston M. Hall  
by attorney.

Southgate & Hawley

W.M. C. 1937

## UNITED STATES PATENT OFFICE

2,075,281

## SMOKER'S PIPE

Preston M. Hall, Worcester, Mass.

Application November 18, 1933, Serial No. 698,661

2 Claims. (Cl. 131—12)

This invention relates to pipes for use by smokers of tobacco.

It is the general object of my invention to provide a pipe for such purposes which is formed 5 from a novel and improved composition in which tobacco enters as an important constituent.

More specifically, my invention relates to a pipe 10 made of tobacco combined with a natural or synthetic resin to form a hard and strong material particularly adapted for its intended purpose.

My invention further relates to arrangements and combinations of parts which will be herein-after described and more particularly pointed 15 out in the appended claims.

A preferred form of the invention is shown in the drawing, in which

Fig. 1 is a side elevation of a pipe embodying 20 my invention;

Fig. 2 is a partial sectional side elevation thereof, and

Fig. 3 is a plan view of a mold in which my improved pipe may be formed.

Referring to the drawing, I have shown a 25 pipe comprising a bowl 10, a stem portion 11, a mouthpiece 12 and a band 13. The bowl is provided with the usual recess 14 to receive the tobacco, and the stem 11 and mouthpiece 12 are provided with an air passage 15, as usual in such 30 constructions.

The band 13 may be of substantial width and overlaps the reduced abutting end portions of the stem 11 and mouthpiece 12.

It will be understood that my invention may 35 be embodied in many shapes and styles of pipes, and that the representation of a pipe in the drawing of this application is illustrative only.

In constructing my improved pipe, I take 40 tobacco which has been thoroughly dried and reduce the same to the form of small fragments or grains. I find it particularly desirable to use tobacco stems in the manufacture of my improved pipe, as these stems contain less nicotine than the ordinary tobacco and also contain very little, if any, of the sweetening or molasses-like 45 substance found in other parts of the leaf. The stems are also largely a waste product, and use of the stems correspondingly reduces the cost of 50 manufacture.

I first thoroughly mix the grains or fragments 55 of tobacco with a natural or synthetic resin in a liquid state and preferably containing approximately sixty percent of volatile matter. I then place the material in an oven where it is dried at

relatively low heat, preferably not substantially exceeding 175° F.

After being thus dried, the tobacco grains are 5 easily separated and are found to be coated with the resinous material, and a considerable quantity of this resinous material may be absorbed by the grains.

Having prepared the tobacco grains as above 10 described, I fill a suitable mold with the grains and thereafter apply a heavy pressure thereto, following which I heat the mold and material to about 300° F., at which heat the resinous material first melts and then fills all the recesses of 15 the mold and the spaces between the grains of tobacco.

The next effect of the heat and pressure is to 20 polymerize the resinous material which, after cooling, is found to be very hard and strong. After this process is complete, the pipe may be easily removed from the mold, as the material 25 tends to shrink slightly during the heating process.

The pressure used may vary within rather wide 30 limits but a pressure of fifteen hundred to five thousand pounds per square inch will usually be found satisfactory. The proportions of tobacco and resinous material may also be varied, but a ratio of one part of tobacco to one part of liquid resinous material is recommended.

If difficulty is encountered by the sticking of 35 the material to the molds, a small amount of some such lubricating substance as stearic acid may be added to prevent such sticking. Usually one percent of stearic acid will be sufficient.

In certain cases and for certain types of pipes 40 it may also be advisable to add a small proportion, possibly five to seven percent, of some fibrous material to the mixture to increase the strength thereof. Short cotton or linen fibers are suitable for this purpose.

In Fig. 3, I have shown a portion of a mold in 45 which my improved pipe may be produced. This mold comprises a block 20 having a recess 21 therein and having a core 22 for the bowl and a second core 23 for the air passage.

The molds are so constructed that the cores may be removed with the pipe and afterwards withdrawn therefrom, or they may be withdrawn from the mold before the pipe is removed therefrom. The upper part of the mold and the means for applying pressure thereto are not shown in the drawing but may be of any usual construction.

A pipe constructed as above described is found 50 to be particularly well adapted for its intended 55

uses, the embodiment of the grains of tobacco in the pipe produce an attractive appearance, and the article may be economically manufactured, largely from what is at present waste material.

- 5 5 The pipe requires less "breaking-in" than the ordinary pipe and gives what smokers term a "sweet smoke".

In the claims the term "resin" is to be understood as including both natural and synthetic 10 resins.

Having thus described my invention and the advantages thereof, I do not wish to be limited to the details herein disclosed, otherwise than as set forth in the claims, but what I claim is:—

- 15 1. As an article of manufacture, a smoker's pipe bowl formed of a compressed mixture of thorough-

ly dried tobacco and a synthetic resin, said mixture having the characteristics of becoming a hardened strong substance under pressure limits between 1500 and 5000 pounds per square inch when said material is at a temperature of about 300° F. 5

2. As an article of manufacture, a smoker's pipe bowl formed of a compressed mixture of thoroughly dried tobacco and a synthetic resin, said mixture having the characteristics of becoming a hardened strong substance under pressure limits between 1500 and 5000 pounds per square inch when said material is at a temperature of about 300° F. and said mixture consisting of approximately one part of tobacco to one part of the 10 synthetic resin. 15

PRESTON M. HALL.